

## UNITED STATES PATENT OFFICE

2,153,619

## PRODUCTION OF PHOTOGRAPHS IN BLUE-BLACK TONES

Hans Fricke, Wolfen, Kreis Bitterfeld, and Emil Joachim Birr, Bitterfeld, Germany, assignors to Agfa Ansco Corporation, Binghamton, N. Y., a corporation of New York

No Drawing. Application June 13, 1938, Serial No. 213,448. In Germany June 19, 1937

6 Claims. (Cl. 95—88)

Our present invention relates to the production of photographs in blue-black tones.

Various agents for the production of photographs from silver chloride and silver chloride-bromide emulsions in blue-black tones are already known. For this purpose for example, quinine and benztriazole are used. These agents, however, hardly affect the resulting tone in the development of silver bromide. In order to displace the tone towards the blue in the case of such emulsions a condensation product of cystine and formaldehyde has been proposed, but this has the drawback that with a long development it causes fogging.

15 It is one object of our invention to provide a process of producing photographs in blue-black tones which overcomes the disadvantages above cited.

Another object of the invention is the provision of a process of producing such blue-black pictures in which a dialkylated 3-alkyl-2-thiohydantoin is present during development.

Yet another object is to provide a process for the production of such pictures by using a dialkylated 3-alkylene-2-thiohydantoin.

Further objects and advantages of the invention are set forth in the following disclosure.

The novel agent may be added to the developing bath or introduced before the development, for example as an addition to the emulsion or to the photographic material. The incorporation of the agent in the emulsion may be carried out by adding it either to the raw material or to the emulsion in any desired stage in its manufacture or by bathing the finished emulsion layer before exposure in a solution of the agent. The agent may, however, be incorporated in the emulsion support, the subbing layer, sub-layer, backing layer or protecting layer, the barytage, the size for the paper on which the emulsions may be coated or the paper pulp. The quantity of material to be added is in all cases advantageously ascertained by preliminary experiment, whereby the optimum quantity can readily be found. The decisive condition for effectiveness of the agents is that they shall be present during development; it being immaterial whether they are already present before the development or whether they reach the developer from the photographic material or come in contact therewith in the emulsion layer only during the development.

The effect of the dialkylated thiohydantoins was not to be foreseen since it is known that un-

substituted thiohydantoins present in the developer cause fogging.

The invention is illustrated by the following examples.

Example 1

To a developer for developing silver bromide paper there is added 0.075 gram of 3.5.5'-trimethyl-2-thiohydantoin per liter of developer. 3.5.5'-trimethyl-2-thiohydantoin is obtained as follows: 11.8 grams of  $\alpha$ -amino-insobutyric acid are neutralized by a solution of potassium hydroxide of 50 per cent strength and heated with an alcoholic solution of 8 grams of methyl mustard oil. The alcohol is then evaporated and the whole heated with hydrochloric acid for a short time. 15 The product thus obtained is recrystallized from water.

Example 2

To 1 kilo of a positive emulsion ready for pouring is added an aqueous solution of 40 mgs. of 3.5.5'-trimethyl-2-thiohydantoin.

Example 3

To a developer for developing a picture copied on silver bromide is added 0.1 gram of 3-ethyl-5.5'-dimethyl-2-thiohydantoin per liter of developer ready for use. 3-ethyl-5.5'-dimethyl-2-thiohydantoin is produced analogous to the manner described in Example 1. Instead of methyl mustard oil there is used ethyl mustard oil.

Example 4

To a positive emulsion ready for pouring is added an aqueous solution of 3-allyl-5.5'-dimethyl-2-thiohydantoin which is obtained analogous to the method described in Example 1; instead of methyl mustard oil it is caused allyl mustard oil to react.

Example 5

To a positive emulsion ready for pouring is added an aqueous solution of 3-allyl-5.5'-dimethyl-2-thiohydantoin which is obtained analogous to the method described in Example 1; instead of methyl mustard oil it is caused allyl mustard oil to react.

We claim:

1. In a process for producing developed silver pictures in blue-black tones from silver halide emulsions, the improvement which comprises developing said silver halide emulsions in the presence of a member selected from the group consisting of dialkylated 3-alkyl-2-thiohydantoins and dialkylated 3-alkylene-2-thiohydantoins.

2. In a process for producing developed silver

- 5 pictures in blue-black tones from silver halide emulsions, the improvement which comprises developing said silver halide emulsions in the presence of 3,5,5'-thiomethyl-2-thiohydantoin.
- 5 3. In a process for producing developed silver pictures in blue-black tones from silver halide emulsions, the improvement which comprises developing said silver halide emulsions in the presence of 3-ethyl-5-5'-dimethyl-2-thiohydantoin.
- 10 4. In a process for producing developed silver pictures in blue-black tones from silver halide emulsions, the improvement which comprises developing said silver halide emulsions in the presence of 3-allyl-5,5'-dimethyl-2-thiohydantoin.
5. A photographic material comprising a silver halide emulsion layer containing a member selected from the group consisting of dialkylated 3-alkyl-2-thiohydantoins and dialkylated 3-allyl-2-thiohydantoins.
- 5 6. A photographic developer comprising developing agents and a member selected from the group consisting of dialkylated 3-alkyl-2-thiohydantoins and dialkylated 2-allyl-2-thiohydantoins.

10 HANS FRICKE.

EMIL JOACHIM BIRR.